

# United States Patent [19]

Masuhara et al.

[11] Patent Number: 4,695,516

[45] Date of Patent: Sep. 22, 1987

[54] HEAT RESISTANT PRECOATED STEEL SHEET AND PROCESS FOR THE PRODUCTION THEREOF

[75] Inventors: Kenichi Masuhara; Kazuo Yamayoshi; Kouji Wakabayashi, all of Chiba, Japan

[73] Assignee: Nissin Steel Co., Ltd., Tokyo, Japan

[21] Appl. No.: 825,263

[22] Filed: Feb. 3, 1986

[30] Foreign Application Priority Data

Feb. 2, 1985 [JP] Japan 60-18985

[51] Int. Cl.<sup>4</sup> B05D 7/04; B05D 7/16

[52] U.S. Cl. 428/623; 148/6.2; 181/244; 427/409; 427/419.5; 428/624; 428/628; 428/632; 428/653

[58] Field of Search 181/244, 246, 256; 428/624, 623, 632, 628, 653, 658, 409, 419.5; 148/6.2

[56] References Cited

FOREIGN PATENT DOCUMENTS

1179558 12/1984 Canada 427/409  
0148718 11/1983 European Pat. Off. 427/409

240956 11/1985 Japan 427/409

Primary Examiner—L. Dewayne Rutledge

Assistant Examiner—George Wyszomierski

Attorney, Agent, or Firm—Wenderoth, Lind & Ponack

[57] ABSTRACT

A heat resistant precoated steel sheet suitable for use in the manufacture of a muffler of an automobile exhaust gas system comprising:

a hot dip aluminized steel sheet,

a chromate pretreatment layer formed on at least one surface of said hot dip aluminized steel sheet and having a chromium pick-up of 10 to 50 mg/m<sup>2</sup>, a primer coat formed on said pretreatment layer and comprising a cured polyamide imide resin and 8 to 52 parts by weight, based on 100 parts by weight of said resin, of strontium chromate intimately admixed with said resin, and

a top coat formed on said primer coat and comprising a cured polyamide imide resin and 8 to 32 parts by weight, based on 100 parts by weight of said resin, of aluminum scale intimately admixed with said resin.

12 Claims, 2 Drawing Figures



F I G. 1



F I G. 2



**HEAT RESISTANT PRECOATED STEEL SHEET  
AND PROCESS FOR THE PRODUCTION  
THEREOF**

The present invention relates to a precoated steel sheet having excellent heat resistance, corrosion resistance and formability suitable for use in the manufacture of a muffler for an automobile exhaust gas system and to a process for the production thereof.

As a muffler for an automobile exhaust gas system, use has been made of one shaped from a hot dip aluminized steel sheet having excellent heat resistance and corrosion resistance. However, the muffler is repeatedly subjected to corrosive heat cycles in that it is exposed to a hot exhaust gas containing moisture and corrosive materials at the time the engine is operating, and when the engine is stopped and the muffler is allowed to cool, or at the time the engine is started when the muffler is still cool, the moisture and corrosive materials are condensed and stay in it. For this reason a muffler simply shaped from a hot dip aluminized steel sheet has become suffered from a disadvantage in that it is corroded within a short period of time and must be replaced.

To overcome such a disadvantage, depending upon the nature of the muffler, it has been proposed to use as a material to fabricate the muffler a hot dip aluminized steel sheet having on at least one surface thereof, a painted organic film, and to shape it into the muffler so that the painted film constitutes the inside surface of the muffler. However prior art precoated steel sheet products are still unsatisfactory. Because the heat resistance of the painted film is insufficient, the film is partly peeled off by the action of the exhaust gas, and the corrosion proceeds through the peeled part.

On the other hand there is a recent tendency to color the outside surface of the muffler, especially in black, to improve the appearance. This coloring is normally carried out by coating a preshaped muffler with a paint of a general composition to form a coating of a desired color. In addition to the unsatisfactory corrosion resistance of the product, there is a disadvantage in that the procedure requires, because of post-coating, a series of steps of degreasing, pretreatment, painting, curing and cooling for every muffler.

Accordingly, an object of the invention is to provide a precoated steel sheet, which can be directly shaped into a muffler, and which exhibits, when used as a muffler, superior heat resistance and corrosion resistance compared to those made of precoated steel sheets heretofore available.

A special object of the invention is to provide a precoated steel sheet suitable for use in the manufacture of an automobile muffler, which has beneficial properties as mentioned above and is colored in black on that surface which will constitute the outside surface of the muffler.

Another object of the invention is to provide a process for the production of the precoated steel sheets as mentioned above suitable for use in the manufacture of an automobile muffler.

According to the invention, there is provided a precoated steel sheet suitable for use in the manufacture of a muffler of an automobile exhaust gas system comprising:

a hot dip aluminized steel sheet,

5 a chromate pretreatment layer formed on at least one surface of said hot dip aluminized steel sheet and having a chromium pick-up of 10 to 50 mg/m<sup>2</sup>, a primer coat formed on said pretreatment layer and comprising a cured polyamide imide resin and 8 to 52 parts by weight, based on 100 parts by weight of said resin, of strontium chromate intimately admixed with said resin, and a top coat formed on said primer coat and comprising a cured polyamide imide resin and 8 to 32 parts by weight, based on 100 parts by weight of said resin, of aluminum scale intimately admixed with said resin.

10 The invention further provides a precoated steel sheet suitable for use in the manufacture of a muffler of an automobile exhaust gas system comprising:

a hot dip aluminized steel sheet, a chromate pretreatment layer formed on each surface of said a hot dip aluminized steel sheet and having a chromium pick-up of 10 to 50 mg/m<sup>2</sup>, a primer coat formed on said pretreatment layer and comprising a cured polyamide imide resin and 8 to 52 parts by weight, based on 100 parts by weight of said resin, of strontium chromate intimately admixed with said resin,

15 a top coat formed on one of the primer coats and comprising a cured polyamide imide resin and 8 to 32 parts by weight, based on 100 parts by weight of said resin, of aluminum scale intimately admixed with said resin, and

20 a black top coat on the other primer coat and comprising a cured polyamide imide resin having intimately admixed therewith 1.5 to 5 parts by weight of aluminum scale, 30 to 40 parts by weight of a calcined black pigment and 4 to 6 parts by weight of silica powder, based on 100 parts by weight of said resin.

25 The invention still further provides a process for the production of a precoated steel sheet suitable for use in the manufacture of a muffler of an automobile exhaust gas system comprising the steps of:

30 treating a hot dip aluminized steel sheet, the surfaces of which have been cleaned, with a chromic acid solution to form a chromate pretreatment layer having a chromium pick-up of 10 to 50 mg/m<sup>2</sup> on at least one surface of said hot dip aluminized steel sheet,

35 applying onto said pretreatment layer a primer coat paint comprising a polyamide imide resin having a molecular weight of from about 2000 to 7000 dissolved in a solvent and 8 to 52 parts by weight, based on 100 parts by weight of said resin, of strontium chromate intimately admixed with said resin, and curing the primer coat paint at a temperature of from 260° to 320° C. to form a primer coat, and

40 applying onto said primer coat a top coat paint comprising a polyamide imide resin having a molecular weight of from about 2000 to 7000 dissolved in a solvent and 8 to 32 parts by weight, based on 100 parts by weight of said resin, of aluminum scale intimately admixed with said resin, and curing the top coat paint at a temperature of from 260° to 320° C. to form a top coat.

45 The invention further provides a process for the production of a precoated steel sheet suitable for use in the manufacture of a muffler of an automobile exhaust gas system comprising the steps of:

treating a hot dip aluminized steel sheet, the surfaces of which have been cleaned, with a chromic acid solution to form a chromate pretreatment layer having a chromium pick-up of 10 to 50 mg/m<sup>2</sup> on each surface of said hot dip aluminized steel sheet, applying onto said pretreatment layer a primer coat paint comprising a polyamide imide resin having a molecular weight of from about 2000 to 7000 dissolved in a solvent and 8 to 52 parts by weight, based on 100 parts by weight of said resin, of strontium chromate intimately admixed with said resin, and curing the primer coat paint at a temperature of from 260° to 320° C. to form a primer coat, and applying onto one of said primer coats a top coat paint comprising a polyamide imide resin having a molecular weight of from about 2000 to 7000 dissolved in a solvent and 8 to 32 parts by weight, based on 100 parts by weight of said resin, of aluminum scale intimately admixed with said resin, while applying onto the other of said primer coats a black top coat paint comprising a polyamide imide resin having a molecular weight of from about 2000 to 7000 dissolved in a solvent and having intimately admixed therewith 1.5 to 5 parts by weight of aluminum scale, 30 to 40 parts by weight of a calcined black pigment and 4 to 6 parts by weight of silica powder, based on 100 parts by weight of said resin, and curing the top coat paints at a temperature of from 260° to 320° C. to form top coats.

The invention will now be described with reference to the attached drawings, in which:

FIG. 1 is an enlarged cross-section of a precoated steel sheet in accordance with the invention having coated layers on one surface thereof; and

FIG. 2 is an enlarged cross-section of a precoated steel sheet in accordance with the invention having coated layers on both surfaces thereof.

As shown in FIG. 1, the precoated steel sheet in accordance with the invention comprises a hot dip aluminized steel sheet 1, a chromate pretreatment layer 2 formed on at least one surface of said steel sheet 1, a primer coat 3 formed on said pretreatment layer 2 and a top coat 4 formed on said primer coat 3.

A suitable hot dip aluminized steel sheet has 30 to 80 g/m<sup>2</sup> of coated metal, total in both surfaces, with Si content of 6 to 9% by weight, and a thickness of 0.4 to 1.6 mm.

The precoated steel sheet in accordance with the invention has a chromate pretreatment layer 2 formed on at least one surface of the hot dip aluminized steel sheet 1. This pretreatment layer 2 serves to improve adhesion between the metal and primer coats, thereby to enhance the corrosion resistance of the precoated steel sheet. The formation of the layer 2 can be carried out by treating a hot dip aluminized steel sheet, the surfaces of which have been cleaned, with a chromic acid solution. While solution comprising chromic acid,

phosphoric acid and acidic sodium fluoride, such as those described in British Patent No. 830,405 are suitable, other known chromate pretreatment solutions may also be used. Whatever chromate pretreatment solutions are used, it is essential to control conditions of the treatment so that a chromate pretreatment layer having a chromium pick-up of 10 to 50 mg/m<sup>2</sup> may be formed. If the chromium pick-up is substantially lower than 10 mg/m<sup>2</sup>, an appreciable improvement of the adhesion between the metal and primer coats and the corrosion resistance of the product will not be achieved. On the other hand it is frequently observed that the primer coat tends to bulge or peel off in the presence of moisture, as the chromium pick-up exceeds 50 mg/m<sup>2</sup>. The hot dip aluminized steel sheet taken from the chromic acid solution is washed with hot water, e.g. at a temperature of from 60° to 80° C., e.g. for about 10 seconds, squeezed with rolls and dried with hot air e.g. at a temperature of 100° C.

The precoated steel sheet in accordance with the invention comprises on the so formed chromate pretreatment layer 2 a primer coat 3 comprising a cured polyamide imide resin and 8 to 52 parts by weight, based on 100 parts by weight of said resin, of strontium chromate intimately admixed with said resin. The formation of the primer coat 3 may be carried out by applying onto the pretreatment layer 2 a primer coat paint followed by curing the same at a temperature of from 260° to 320° C. The primer coat paint comprises a polyamide imide resin having a molecular weight of from about 2000 to 7000, preferably about 3000 to 6000, dissolved in a solvent and 8 to 52 parts by weight, based on 100 parts by weight of said resin, of strontium chromate, SrCrO<sub>4</sub>, intimately admixed with said resin. For the corrosion resistance intended herein at least 8 parts by weight, based on 100 parts of the resin, of strontium chromate must be present in the primer coat, and in turn in the primer coat paint. However, the presence of strontium chromate in the primer coat 3 in an amount substantially in excess of 52 parts by weight based on 100 parts by weight of the resin must be avoided, because such an excessive addition not only renders the primer coat 3 porous to deteriorate its properties, but also adversely affects the adhesion between the metal and primer coats to thereby lower the corrosion resistance of the product.

The polyamide imide resins suitable for use in the primer coat paint are polymers having amide linkages and imide linkages, which are soluble in a particular solvent used, preferably N-methyl-2-pyrrolidone, and have a molecular weight of 2000 to 7000, preferably 3000 to 6000. Preferred polyamide imide resins are aromatic polymers having repeating units of the general formula I, II or III, which constitute at least 70% by mole of the polymer chain, with the remaining 30% by mole or less of the polymer chain being represented by repeating units of the general formula IV or V.



-continued



(III)



(IV)

(V)



In the above formulae, Ar independently represents a divalent aromatic group selected from



wherein X represents



Incidentally, a part of the imide linkages shown in the formulae I, II, III and V above may be in the state of its precursor before ring closure, that is the amide linkage. Some of the preferred polyamide imide resins are described in Japanese Patent Publication No. 57-61775 and Japanese Patent Laid-open application No. 59-8755.

Some of them are commercially available. Especially preferred polyamide imide resins are those in which at least 85% by mole of the polymer chain is represented by the repeating unit of the formula III above, wherein all of the Ar are o-phenylene, and which have a molecular weight of about 3000 to 6000.

As the solvent, N-methyl-2-pyrrolidone is most preferred, but other organic polar solvents, including, for example, dimethylformamide, dimethylacetamide, dimethylsulfoxide and hexamethylphosphoamide may also be used, so far as they dissolve the polyamide imide resin used.

The primer coat should preferably have a thickness of 3 to 8  $\mu\text{m}$  on dry basis. The primer coat paint is conveniently applied by a roll coating method, and the consistency of the primer coat paint is adjusted so that the above-mentioned thickness on dry basis may be obtained by the roll coating method. For the above mentioned dry thickness, the curing time can be as short as about 60 seconds or less, for example, 40 seconds or less, at a curing temperature (temperature of atmosphere in the curing furnace) of from 260° to 320° C.

The precoated steel sheet according to the invention further comprises a top coat 4 on the so formed primer coat 3, the top coat 4 comprising a cured polyamide imide resin and 8 to 32 parts by weight, based on 100 parts by weight of said resin, of aluminum scale intimately admixed with said resin. The formation of the top coat may be carried out by applying a top coat paint

15

onto the primer coat 3 followed by curing the same at a temperature of 260° to 320° C.

The top coat paint comprises a polyamide imide resin having a molecular weight of from about 2000 to 7000, 20 preferably about 3000 to 6000, dissolved in a solvent and 8 to 32 parts by weight, based on 100 parts by weight of said resin, of aluminum scale intimately admixed with said resin. For the purpose of the invention 8 to 32 parts by weight, based on 100 parts by weight of 25 the resin, of aluminum scale must be present in the top coat 4, and in turn in the top coat paint. The size and shape of preferred aluminum scale are such that it has an average size (average length of the longest side) of 15 to 35  $\mu\text{m}$  and at least 99% may pass through a sieve of JIS 30 325 mesh, and that it has an average aspect ratio (ratio of the longer diameter to the shorter diameter) of 10 to 50. Such aluminum scale serves to enhance the heat resistance and adhesion of the painted films, and in addition, it further protects the aluminum coated layer by physical shielding effect due to its scale shape. To appreciably achieve such results, the addition of at least 8 parts by weight, based on 100 parts by weight of the resin, of aluminum scale is required. But addition of aluminum scale substantially in excess of 32 parts by weight, based on 100 parts by weight of the resin, must be avoided, or otherwise the resin painted films will become brittle, leading to a poor formability of the product.

The polyamide imide resin and solvent used in the top 40 coat paint may be the same as used in the primer coat composition. The manner of application and the curing temperature may also be the same as described above. However, the thickness of the top coat layer 4 on dry basis should preferably be thicker than that of the prime coat layer 3, and can be for example about 8 to 20  $\mu\text{m}$ . Owing to the thicker dry thickness of the top coat layer 4, it is preferred to use a slightly higher consistency and a somewhat longer curing time (for example 60 to 90 seconds) for the top coat paint than for the primer coat paint. The coated strip which has left the curing furnace may be cooled with sprayed water, squeezed with rolls and dried with hot air, for example, at a temperature of about 50° C.

That side of the precoated steel sheet in accordance 55 with the invention shown in FIG. 1, which is not shown in that Figure, can be the surface of the aluminum hot dip coated steel sheet 1 as such, or in the state that the chromate pretreatment layer 2 only has been formed on the surface of the aluminum hot dip coated steel sheet 1, or in the state that via the pretreatment layer 2 one or two layers of suitable heat resistant resins have been formed on the surface of the hot dip aluminized steel sheet 1.

Alternatively, the precoated steel sheet in accordance with the invention may comprise, as shown in FIG. 2, the hot dip aluminized steel sheet 1, as described above, having on each surface thereon, via a chromate pretreatment layer 2, as described above, both the primer and top coats, as described above. In the precoated steel sheet shown in FIG. 2, the two pretreatment layer 2, two primer coats 3, and two top coats 4 may be respectively the same and may be respectively formed at the same time in the manner as described above.

When a muffler with the outside surface colored in black is desired, use may be made of a precoated steel sheet in accordance with the invention comprising a hot dip aluminized steel sheet 1, as described above, having formed on one surface thereof a chromate pretreatment layer 2, a primer coat 3 and a top coat 4, which layers are the same as described above, and also having formed on the other surface thereof a chromate pretreatment layer 2, a primer coat 3, which layers are the same as described above, and a top coat containing a black pigment. Such a precoated steel sheet in accordance with the invention may be shaped into a muffler so that the black top coat layer may constitute the outside surface of the muffler. The black top coat layer may be generally a coated layer of a cured heat resistant resin. Optimum results have been obtained, however, by using a polyamide imide resin, as described above, as the heat resistant resin, and a calcined black pigment, such as graphite, having a relatively large specific surface area ranging between 100 and 1000 m<sup>2</sup>/mg, as the coloring agent, and by incorporating a small amount of aluminum scale as described above and a small amount of silica powder as a matting agent. More precisely, the best results have been obtained by a black top coat comprising a cured polyamide imide resin having intimately admixed therewith 1.5 to 5 parts by weight of aluminum scale, 30 to 40 parts by weight of a calcined black pigment and 4 to 6 parts by weight of silica powder, based on 100 parts by weight of said resin. The precoated steel sheet in accordance with the invention having such a preferred black coating may be prepared by forming on both surfaces of the hot dip aluminized steel sheet 1 the chromate pretreatment layers 2 and the prime coats 3 in the manner as described above, and applying onto one of said primer coats a top coat paint comprising a polyamide imide resin having a molecular weight of from about 2000 to 7000 dissolved in a solvent and 8 to 32 parts by weight, based on 100 parts by weight of said resin, of aluminum scale intimately admixed with said resin, while applying onto the other of said primer coats a black top coat paint comprising a polyamide imide resin having a molecular weight of from about 2000 to 7000 dissolved in a solvent and having intimately admixed therewith 1.5 to 5 parts by weight of aluminum scale, 30 to 40 parts by weight of a calcined black pigment and 4 to 6 parts by weight of silica powder, based on 100 parts by weight of said resin, and baking the compositions at a temperature of from 260° to 320° C. to form top coat layers. Both the top coat paint may be applied in the manner described above, and may be cured, cooled and dried at the same time in the manner as described above.

The invention will be further described by the following Examples.

#### EXAMPLE 1

An aluminum hot dip coated steel sheet (200 mm wide, 300 mm long and 0.6 mm in thickness) and 40

g/m<sup>2</sup> (total on both surfaces) of the coating metal with 6% by weight of Si was immersed for about 10 seconds in "Ridoline 35 N1" (an alkaline degreasing solution, supplied by Nippon Paint Co., Ltd.) having the ingredient concentration adjusted at 4% by weight and maintained at a temperature of 60° C., taken out of the liquid, and washed with hot water at about 70° C. for about 10 seconds.

A mixed solution of "Arozin #407" having the ingredient concentration adjusted at 4% by weight and "Arozin #47" having the ingredient concentration adjusted to 0.6% by weight was maintained at a temperature of 60° C. The "Arozin #407" and "Arozin #47" are acidic chromate formation liquids of chromic acid-phosphoric acid series, supplied by Nippon Paint Co., Ltd. The hot dip aluminized steel sheet, the surfaces of which had been cleaned, was immersed in the mixed solution for about 10 seconds, whereby chromate pretreatment layers, each having a chromium pick-up of about 25 mg/m<sup>2</sup>, were formed on both surfaces of the aluminum coated steel sheet. The sheet taken out of the pretreatment solution, was washed with hot water at about 70° C. for about 10 seconds and dried with hot air at about 100° C. In this way many pretreated sheets were prepared.

To a polyamide imide resin varnish (a solution of a polyamide imide resin having an average molecular weight of about 4500 in N-methyl-2-pyrrolidone) strontium chromate in an amount indicated in Table 1 was added, and the resultant mixture was diluted under stirring with an appropriate amount of N-methyl-2-pyrrolidone to prepare each primer coat paint. It was applied by a roll coating method onto one surface of the pretreated hot dip aluminized steel sheet, and cured for about 40 seconds in a conveyor-oven maintained at a temperature of 280° C., to form a primer coat having a dry thickness of about 4 μm.

To the above-mentioned polyamide imide resin varnish, non-leaving type aluminum scale (more than 99% by weight of which was capable of passing through a sieve of JIS 325 mesh) having an average size of about 25 μm and an average aspect ratio of about 20, in an amount indicated in Table 1 was added, and the resultant mixture was diluted under stirring with an appropriate amount of N-methyl-pyrrolidone to prepare each top coat paint. It was applied by a roll coating method onto the primer coat, and cured for about 80 seconds in a conveyor-oven maintained at a temperature of 280° C., to form a top coat having a dry thickness of about 12 μm. The sheet removed from the oven was cooled by spraying water, squeezed with rolls and dried with warm air of a temperature of about 50° C.

The coated steel sheet samples were tested for the heat resistance, corrosion resistance and formability, and results were estimated in accordance with the following manner and are shown in Table 1.

##### (1). Heat resistance

The sample was heated in a hot air circulating dryer at a predetermined temperature indicated in Table 1 for 200 hours, conditioned at 20° C. and 60%RH for 24 hours, and then subjected to an adhesion test in accordance with JIS-G3312. The heat resistance of the sample was estimated according to the following rating.

- A: Completely no peeling of the painted film
  - B: Slight peeling of the painted film
  - C: Considerable peeling of the painted film
  - D: Remarkable peeling of the painted film
- (2). Corrosion resistance

A 500 hours Salt Spray test in accordance with JIS-Z2371 (SST) and a 500 hours Humidity test in accordance with JIS-K224(BB) were carried out. The corrosion resistance of the sample was estimated according to the following rating.

- A: Completely no bulging of the coating painted film and occurrence of no rust
- B: Slight bulging of the painted film and occurrence of slight rust
- C: Considerable bulging of the painted film and occurrence of considerable rust
- D: Remarkable bulging of the painted film and occurrence of remarkable rust

(3). Formability

The sample was bent by an angle of 180 degrees in such a manner that a stack of 4 sheets, each having the same thickness as the sample, was sandwiched between the bent halves of the sample. The stressed portion of the sample was subjected to an adhesion test in accordance with JIS-3312. The formability of the sample was estimated according to the following rating.

10

EXAMPLE 2

In this example, the heat resistance, corrosion resistance and formability of various black colored coatings were examined.

Graphite powder having a specific surface area of 200 m<sup>2</sup>/mg and aluminum scale as used in Example 1, respectively in amounts as indicated in table 2, were added to a varnish of polyamide imide resin as used in Example 1 and the resultant mixture was diluted under stirring with an appropriate amount of N-methyl-2-pyrrolidone to prepare each top coat paint.

Using the top coat paints so prepared and primer coat paints suitable for the provision of primer coats indicated in Table 2, the procedure as described in Example 1 was followed to prepare samples to be tested.

The samples so prepared were tested for the heat resistance, corrosion resistance and formability as in Example 1. The results are shown in Table 2.

TABLE 2

| Run No. | Primer coat        |                                | Top coat              |                            |                      | Heat resistance    |          |         | Corrosion resistance |       | Formability |              |
|---------|--------------------|--------------------------------|-----------------------|----------------------------|----------------------|--------------------|----------|---------|----------------------|-------|-------------|--------------|
|         | Resin 100 wt. part | Strontium chromate (wt. parts) | Resin (100 wt. parts) | Aluminum scale (wt. parts) | Graphite (wt. parts) | Silica (wt. parts) | 200 hrs. |         |                      | S.S.T | B.B.T       | 180° 4t bend |
|         |                    |                                |                       |                            |                      |                    | 250° C.  | 270° C. | 300° C.              |       |             |              |
| 1       | Polyamide imide    | 20                             | Polyamide imide       | 2                          | 33                   | 4                  | A        | B       | B                    | B     | B           | A            |
| 2       | Polyamide imide    | 20                             | Polyamide imide       | 2                          | 37                   | 4                  | A        | B       | B                    | B     | B           | A            |
| 3       | Polyamide imide    | 20                             | Polyamide imide       | 4                          | 33                   | 4                  | A        | A       | B                    | B     | B           | A            |
| 4       | Polyamide imide    | 20                             | Polyamide imide       | 4                          | 37                   | 4                  | A        | A       | B                    | B     | B           | A            |
| 5       | Polyamide imide    | 30                             | Polyamide imide       | 2                          | 33                   | 4                  | A        | B       | B                    | B     | B           | A            |
| 6       | Polyamide imide    | 30                             | Polyamide imide       | 2                          | 37                   | 4                  | A        | B       | B                    | B     | B           | A            |
| 7       | Polyamide imide    | 30                             | Polyamide imide       | 4                          | 33                   | 4                  | A        | A       | B                    | B     | B           | A            |
| 8       | Polyamide imide    | 30                             | Polyamide imide       | 4                          | 37                   | 4                  | A        | A       | B                    | B     | B           | A            |
| 9       | Polyamide imide    | 20                             | Polyamide imide       | 2                          | 10                   | 4                  | B        | C       | D                    | B     | B           | A            |
| 10      | Polyamide imide    | 20                             | Polyamide imide       | 2                          | 50                   | 4                  | B        | C       | D                    | B     | C           | D            |
| 11      | Polyamide imide    | 20                             | Polyamide imide       | 0                          | 35                   | 4                  | C        | C       | D                    | C     | C           | A            |
| 12      | Polyamide imide    | 20                             | Polyamide imide       | 7                          | 35                   | 4                  | B        | C       | C                    | B     | B           | C            |
| 13      | Polyamide imide    | 5                              | Polyamide imide       | 3                          | 35                   | 4                  | A        | B       | B                    | D     | C           | A            |
| 14      | Polyamide imide    | 70                             | Polyamide imide       | 3                          | 35                   | 4                  | B        | C       | C                    | C     | C           | C            |
| 15      | Polyamide imide    | 20                             | Polyamide imide       | 3                          | 35                   | 10                 | B        | C       | D                    | C     | C           | D            |

Runs No. 1-8: Black top coat layer recommended herein

Runs No. 9-15: Controls

dance with JIS-3312. The formability of the sample was estimated according to the following rating.

- A: Completely no peeling of the painted film
- B: Very slight peeling of the painted film
- C: Considerable peeling of the painted film
- D: Full peeling of the painted film

The test results are shown in Table 1 together with the composition of the painted film of the tested samples.

What is claimed is:

1. A precoated steel sheet suitable for use in the manufacture of a muffler of an automobile exhaust gas system comprising:
  - 45 a hot dip aluminized steel sheet,
  - a chromate pretreatment layer formed on at least one surface of said hot dip aluminized steel sheet and having a chromium pick-up of 10 to 50 mg/m<sup>2</sup>,
  - 50 a primer coat formed on said pretreatment layer and comprising a cured polyamide imide resin and 8 to

TABLE 1

| Run No. | Primer coat         |                                | Top coat              |                            |                      | Heat resistance    |          |         | Corrosion resistance |       | Formability |              |
|---------|---------------------|--------------------------------|-----------------------|----------------------------|----------------------|--------------------|----------|---------|----------------------|-------|-------------|--------------|
|         | Resin 100 wt. parts | Strontium chromate (wt. parts) | Resin (100 wt. parts) | Aluminum scale (wt. parts) | Graphite (wt. parts) | Silica (wt. parts) | 200 hrs. |         |                      | S.S.T | B.B.T       | 180° 4t bend |
|         |                     |                                |                       |                            |                      |                    | 250° C.  | 270° C. | 300° C.              |       |             |              |
| 1       | Polyamide imide     | 20                             | Polyamide imide       | 10                         | A                    | A                  | A        | B       | A                    | A     | A           | A            |
| 2       | Polyamide imide     | 20                             | Polyamide imide       | 20                         | A                    | A                  | A        | A       | A                    | A     | A           | A            |
| 3       | Polyamide imide     | 20                             | Polyamide imide       | 30                         | A                    | A                  | A        | A       | A                    | A     | B           |              |
| 4       | Polyamide imide     | 30                             | Polyamide imide       | 10                         | A                    | A                  | A        | A       | A                    | A     | A           | A            |
| 5       | Polyamide imide     | 30                             | Polyamide imide       | 20                         | A                    | A                  | A        | A       | A                    | A     | A           | A            |
| 6       | Polyamide imide     | 30                             | Polyamide imide       | 30                         | A                    | A                  | A        | A       | A                    | A     | B           |              |
| 7       | Polyamide imide     | 5                              | Polyamide imide       | 20                         | A                    | A                  | A        | D       | C                    | C     | A           |              |
| 8       | Polyamide imide     | 20                             | Polyamide imide       | 5                          | B                    | B                  | D        | C       | B                    | B     | A           |              |
| 9       | Polyamide imide     | 20                             | Polyamide imide       | 45                         | B                    | C                  | D        | B       | C                    | C     | D           |              |
| 10      | Polyamide imide     | 70                             | Polyamide imide       | 20                         | B                    | B                  | C        | C       | C                    | C     | D           |              |

Runs No. 1-6: According to the invention

Runs No. 7-10: Controls

52 parts by weight, based on 100 parts by weight of said resin, of strontium chromate intimately admixed with said resin, and a top coat formed on said primer coat and comprising a cured polyamide imide resin and 8 to 32 parts by weight, based on 100 parts by weight of said resin, of aluminum scale intimately admixed with said resin.

2. The precoated steel sheet in accordance with claim 1 wherein said hot dip aluminized steel sheet has a thickness of 0.4 to 1.6 mm, said primer coat has a thickness of 3 to 8  $\mu\text{m}$ , and said top coat has a thickness of 8 to 20  $\mu\text{m}$ .

3. The precoated steel sheet in accordance with claim 2 wherein said aluminum scale has an average size of 15 to 35  $\mu\text{m}$  and an aspect ratio of from 10 to 50.

4. A precoated steel sheet suitable for use in the manufacture of a muffler of an automobile exhaust gas system comprising:

a hot dip aluminized steel sheet, a chromate pretreatment layer formed on each surface of said a hot dip aluminized steel sheet and having a chromium pick-up of 10 to 50  $\text{mg}/\text{m}^2$ , a primer coat formed on said pretreatment layer and comprising a cured polyamide imide resin and 8 to 52 parts by weight, based on 100 parts by weight of said resin, of strontium chromate intimately admixed with said resin, a top coat formed on one of the primer coats and comprising a cured polyamide imide resin and 8 to 32 parts by weight, based on 100 parts by weight of said resin, of aluminum scale intimately admixed with said resin, and a black top coat on the other primer coat and comprising a cured polyamide imide resin having intimately admixed therewith 1.5 to 5 parts by weight of aluminum scale, 30 to 40 parts by weight of a calcined black pigment and 4 to 6 parts by weight of silica powder, based on 100 parts by weight of said resin.

5. The precoated steel sheet in accordance with claim 4 wherein said hot dip aluminized steel sheet has a thickness of 0.4 to 1.6 mm, said primer coat has a thickness of 3 to 8  $\mu\text{m}$ , and said top coat has a thickness of 8 to 20  $\mu\text{m}$ .

6. The precoated steel sheet in accordance with claim 5 wherein said aluminum scale has an average size of 15 to 35  $\mu\text{m}$  and an aspect ratio of from 10 to 50.

7. The precoated steel sheet in accordance with claim 4 wherein said calcined black pigment has a specific surface area of from 100 to 1000  $\text{m}^2/\text{g}$ .

8. A process for the production of a precoated steel sheet suitable for use in the manufacture of a muffler of an automobile exhaust gas system comprising the steps of:

treating a hot dip aluminized steel sheet, the surfaces of which have been cleaned, with a chromic acid solution to form a chromate pretreatment layer having a chromium pick-up of 10 to 50  $\text{mg}/\text{m}^2$  on at least one surface of said hot dip aluminized steel sheet,

applying onto said pretreatment layer a primer coat paint comprising a polyamide imide resin having a molecular weight of from about 2000 to 7000 dissolved in a solvent and 8 to 52 parts by weight, based on 100 parts by weight of said resin, of strontium chromate intimately admixed with said resin, and curing the primer coat paint at a temperature of from 260° to 320° C. to form a primer coat, and applying onto said primer coat a top coat paint comprising a polyamide imide resin having a molecule weight of from about 2000 to 7000 dissolved in a solvent and 8 to 32 parts by weight, based on 100 parts by weight of said resin, of aluminum scale intimately admixed with said resin, and curing the top coat paint at a temperature of from 260° to 320° C. to form a top coat.

9. The process for the production of a precoated steel sheet in accordance with claim 8 wherein said aluminum scale has an average size of 15 to 35  $\mu\text{m}$  and an aspect ratio of from 10 to 50.

10. A process for the production of a precoated steel sheet suitable for use in the manufacture of a muffler of an automobile exhaust gas system comprising the steps of:

treating a hot dip aluminized steel sheet, the surfaces of which have been cleaned, with a chromic acid solution to form a chromate pretreatment layer having a chromium pick-up of 10 to 50  $\text{mg}/\text{m}^2$  on each surface of said hot dip aluminized steel sheet, applying onto said pretreatment layer a primer coat paint comprising a polyamide imide resin having a molecular weight of from about 2000 to 7000 dissolved in a solvent and 8 to 52 parts by weight, based on 100 parts by weight of said resin, of strontium chromate intimately admixed with said resin, and curing the primer coat paint at a temperature of from 260° to 320° C. to form a primer coat, and applying onto one of said primer coats a top coat paint comprising a polyamide imide resin having a molecular weight of from about 2000 to 7000 dissolved in a solvent and 8 to 32 parts by weight, based on 100 parts by weight of said resin, of aluminum scale intimately admixed with said resin, while applying onto the other of said primer coats a black top coat paint comprising a polyamide imide resin having a molecular weight of from about 2000 to 7000 dissolved in a solvent and having intimately admixed therewith 1.5 to 5 parts by weight of aluminum scale, 30 to 40 parts by weight of a calcined black pigment and 4 to 6 parts by weight of silica powder, based on 100 parts by weight of said resin, and curing the top coat paints at a temperature of from 260° to 320° C. to form top coats.

11. The process for the production of a precoated steel sheet in accordance with claim 10 wherein said aluminum scale has an average size of 15 to 35  $\mu\text{m}$  and an aspect ratio of from 10 to 50.

12. The process for the production of a precoated steel sheet in accordance with claim 10 wherein said calcined black pigment has a specific surface area of from 100 to 1000  $\text{m}^2/\text{g}$ .

\* \* \* \* \*